

## UNITED STATES PATENT OFFICE

2,360,939

## MAGNETIC MATERIALS

Joy F. Dillinger, Riverside, and Arthur N. Ogden, Chicago, Ill., assignors to Western Electric Company, Incorporated, New York, N. Y., a corporation of New York

No Drawing. Application October 21, 1942,  
Serial No. 462,844

## 4 Claims. (Cl. 75—0.5)

This invention relates to magnetic materials and to a method of preparing the same, and more particularly to magnetic materials to be used as stabilizers and a method of preparing the same.

Magnetic bodies comprising compressed, finely divided magnetic material in the form of dust or assembled thin laminations of magnetic material are extensively used as cores for loading coils, filtering coils, transformers and similar transmission apparatus in telephone circuits. The transmission characteristics of such apparatus are subject to variations due to changes in the permeability of the cores with changes in temperature under service conditions. These variations are particularly objectionable in the case of high quality precision circuits.

In order to prevent these variations, a magnetic material, which has a suitable permeability temperature coefficient as compared with that of the core material, may be added to the primary core material to compensate for variations due to temperature. Such a material is generally referred to as a stabilizer.

As described in U. S. Patent 2,158,132, issued to V. E. Legg, May 16, 1939, a magnetic core having a substantially constant permeability over a desired temperature range may be prepared by forming the core from a mixture of a magnetic material such as Permalloy, which may comprise approximately 82% nickel, 16% iron and 2% molybdenum and which has a positive permeability temperature coefficient over the range of temperature from 55° F. to 125° F., and a proper amount of dust of a second magnetic material having a negative permeability coefficient over that temperature range. A magnetic material having such a negative permeability coefficient may comprise approximately 80% nickel, 12% to 13% molybdenum and the rest iron. Such a material, when used with the first described magnetic material, serves as a stabilizer of the permeability of the magnetic core.

Molybdenum tends to oxidize during melting, and the oxide so formed tends to volatilize. This results in a loss of some of the molybdenum, and since a variation in the amount of molybdenum present in the stabilizer of even 1% will result in a change in the Curie point of the stabilizer of approximately 100° F., it will be apparent that the exact permeability temperature coefficient of the stabilizer material will depend largely on the molybdenum present in the final stabilizer dust. Furthermore, an ingot formed from a melt containing a known amount of molybdenum and the other aforementioned materials will have areas of

differing permeability and differing Curie points. This appears to be due to a segregation of molybdenum particles during cooling and appears to be unavoidable even in the most thoroughly mixed melts.

An object of the present invention is to provide an effective and efficient method of obtaining stabilizer materials having predetermined magnetic properties.

10 In accordance with one embodiment of this invention, magnetic material may be powdered and the powder passed through a magnetic separating machine a number of times at increasing temperatures to obtain materials having increasingly higher Curie points.

In accordance with another embodiment of this invention, a powdered magnetic material may be passed a number of times through a magnetic separator under increasing field strengths at a 20 constant temperature to obtain materials having progressively lower Curie points.

Other objects and advantages of this invention will be apparent from the following detailed description.

25 This invention will be described in connection with the production of magnetic materials having Curie points between 55° F. and 125° F. It will be understood, however, that the method of this invention is applicable to the production of magnetic materials having Curie points within any desired feasible range.

In the practice of this invention, an ingot of magnetic material is prepared by melting together approximately 80% nickel, 12% to 13% 35 molybdenum and the rest iron. These materials may be melted together in any suitable furnace to produce an alloy. Melting is carried out in a non-reducing atmosphere, in general, and some compensation must be made for the loss of molybdenum during melting by the addition of extra molybdenum in advance. In practice this loss

40 has been found to amount to not more than .25%. However, because of the considerable effect on the Curie point of the stabilizer material of even 45 a slight change in the amount of molybdenum present, it is desirable to control the amount of molybdenum in the final alloy within very close limits so far as possible.

The ingot is then hot rolled and the fragments 50 reduced to powder. In order to keep contamination due to wear at a minimum, an impact type machine may be used for pulverization and the powder reduced to approximately 400 mesh fineness.

55 In accordance with one embodiment of this in-

vention, the powder so obtained may then be passed through a magnetic separator at a temperature of approximately 50° F. Material, the Curie point of which has been reached will be separated into one group by the separator, while material having a higher Curie point will be separated into another group. The latter group of material is then passed through the separator at a temperature of, for example, 55° F. to obtain magnetic materials having Curie points at approximately 55° F. On successive passes, the temperature may be raised and the process repeated with the material left until materials having a sufficient range of Curie points are obtained. The field strength of the magnetic separator must, of course, be maintained constant and the precise field strength to be used will depend upon the area of the magnetic field and the amount of material being passed thereunder at a given time. By removing in advance material having a Curie point lower than that which it is desired to obtain, in addition materials having lower permeabilities and non-magnetic materials, are substantially removed and, in subsequent passes, the material which will be segregated will be substantially purely magnetic, differing only as to Curie points. It will be apparent that the first separating pass could be made at a high temperature, and thereafter successive passes made at relatively lower temperatures without departing from the spirit or scope of this embodiment of the present invention.

In accordance with another embodiment of this invention, where it is not feasible to control the temperature of the magnetic material as it is passed through the magnetic separator within the close limits required, magnetic materials having varying Curie points may be satisfactorily segregated by maintaining a constant temperature and varying the field strength of the magnetic separator.

The magnetic material is prepared and powdered in the same way as described hereinbefore. The powder so obtained is then heated to a temperature of approximately 180° F., and the heated powder spread out in a very thin layer on the separator belt. The temperature of the material should be so controlled so that the powder on the belt is approximately 140° F. to 170° F. as it falls on the belt. This may be determined by holding a thermometer in the stream of powder as it falls on the belt. The portion of the powder which is discharged on the non-magnetic side of the separator is used for further processing and that portion of powder discharged on the magnetic side is discarded as unsuitable for use as a stabilizing powder in the range of 55° F. to 125° F. This rough preliminary separation of the powder is particularly necessary where materials are to be separated by varying the field strength since even in the most closely controlled melts, materials having varying permeabilities at the same temperature occur, and since materials having Curie points substantially higher than those desired will also occur.

The material which was discharged on the non-magnetic side of the separator is then passed through the magnetic separator several times at a constant temperature, preferably room temperature, starting at a low value of magnetic field strength and increasing the field strength for each successive pass. The field strength may be adjusted either by varying the current passing through the magnetizing coils or by varying

the separation between the magnetic poles of the separator. For the first pass, the field strength should be so adjusted that between 10% and 20% of the material is discharged on the magnetic side of the separator. In successive passes, the field strength should be increased so that approximately 20% of the material is discharged on the magnetic side of the separator in each pass. If the current has been increased to the maximum possible and a large percentage of the material still remains in the non-magnetic portion, the field strength should be further increased by moving the poles closer together.

As a magnetic material approaches its Curie point, its permeability decreases sharply; thus, greater field strength is required in a magnet to attract a material near its Curie point than a material not near its Curie point, assuming the materials are equal in permeability. Thus, in the first pass after the rough separation, the material having the highest Curie point will be discharged on the magnetic side of the separator and, in successive passes, material having Curie points progressively lower will be discharged on the magnetic side of the separator.

It has been found in practice that the accuracy of separation by either embodiment of this invention is substantially the same, the advantage of the former method of separation over the latter described being that the latter will not distinguish between one material which has a low permeability due to its proximity to the Curie point and another which is far removed from its Curie point, but inherently of low permeability, whereas the former will so distinguish. However, in the latter case, by carefully controlling the composition of the melt and by making the rough preliminary separation described, this difficulty is largely obviated.

The magnetic core is then formed by using a small amount of a stabilizer powder comprising particles having a plurality of Curie points over the range of 55° F. to 125° F. Stabilizer materials having more than one Curie point are used so as to stabilize the temperature permeability coefficient over the whole range desired rather than at only one temperature. In practice, before combining portions of the separated groups of magnetic material, it may be desirable to test each group to determine accurately the magnetic characteristics thereof and thereby to determine precisely what proportions of each group to employ to obtain a mixture having the desired properties.

Using permalloy dust, as hereinbefore described, to form a magnetic core insulated, for example, as described in the patent to A. F. Bandur, 2,105,070, issued January 11, 1938, the permeability of a core so formed may be stabilized over a range of temperature from 55° F. to 125° F. by the addition of .2% to 1% stabilizer powder of the type herein described in most cases. The minimum amount of stabilizing powder which will accomplish the desired stabilization is used because of the high hysteresis loss of the stabilizer material.

While but two embodiments of this invention have been shown and described, it will be understood that many changes and modifications may be made therein without departing from the spirit or scope of the present invention.

What is claimed is:

1. A method of forming a stabilizer material for magnetic cores, said material comprising particles having a variety of Curie points, said

method comprising powdering a magnetic material composed of approximately 80% nickel, 12% to 13% molybdenum, and the rest iron, passing the powdered material through a magnetic separator at a temperature lower than the temperature of the lowest desired Curie point and then passing the remaining material through the separator at successively higher temperatures to obtain particles having a variety of Curie points.

2. A method of preparing a stabilizer material for magnetic cores, said material comprising particles having a variety of Curie points, said method comprising powdering a magnetic material composed of approximately 80% nickel, 12% to 13% molybdenum and the rest iron, and successively passing the powdered material through a magnetic separating device at increasing temperatures, the particles the Curie point of which has been reached being discharged on the non-magnetic side of the separator.

3. A method of forming a stabilizer material for magnetic cores, said magnetic material having a variety of Curie points and composed of approximately 80% nickel, 12% to 13% molybdenum and the rest iron, comprising heating 25

ing this heated material through a magnetic separator to remove all material having a Curie point above that temperature, and then successively passing the remaining material through the separator at a lower temperature and under increasing field strengths to obtain materials having varying Curie points.

4. A method of forming a stabilizer composing particles having a variety of Curie points for magnetic cores, comprising heating a comminuted mixture composed of approximately 80% nickel, 12% to 13% molybdenum and the rest iron to a temperature above that of the highest Curie point desired, passing this heated material through a magnetic separator to remove substantially all material having a Curie point above that temperature, successively passing the remaining material through the separator at a lower temperature and under increasing field strengths to obtain materials having varying Curie points, and then recombining portions of the variously separated materials to obtain a stabilizer material having the desired characteristics.

JOY F. DILLINGER.  
ARTHUR N. OGDEN.